

## UNITED STATES PATENT OFFICE

2,626,224

CLEANING OXIDE FROM OXIDIZED  
MOLYBDENUM WIRE

Marie A. Levesque, Peabody, Mass.

No Drawing. Application November 30, 1949,  
Serial No. 130,367

2 Claims. (Cl. 134--3)

1

This invention relates generally to treatment of the surface only of a material with a combination of chemicals with which the material itself reacts, and in particular relates to cleaning oxide from the surface of a metal, which may be for example, molybdenum.

An object of the invention is to clean from the surface of, or otherwise affect the surface of, a material without affecting the body of the material itself. A particular object is to remove oxide from an oxidized molybdenum wire without removing any appreciable amount of the molybdenum wire itself.

A feature of the invention is the dipping of a material into a chemical bath, and then while still wet with the first chemical, dipping it into a second chemical bath.

A particular feature is the dipping of a metal wire into a bath of nitric acid solution and then while the metal is still wet with the nitric acid solution, dipping it into a solution of hydrochloric acid.

Other features, objects and advantages of the invention will be apparent from the following description.

In the use of molybdenum wire in electric lamps and the like, it is desired to have the surface extremely clean of all impurities such as oxides and the like, and in many cases the molybdenum wire as received may have a heavy film of oxide. My invention avoids the considerable corrosive effect which the usual cleaning baths have on the metal itself.

In cleaning oxidized molybdenum wire, for example, according to my invention, I dip the wire in a solution of nitric acid, which may be, for example, 3 parts water and 8 parts nitric acid. Such a solution will have a specific gravity of about 1.15.

After dipping the wire in the nitric acid for about 10 seconds I remove it from that solution and immediately dip it into a solution of hydrochloric acid, the solution being, for example, about 3 parts acid and 8 parts water, having a specific gravity, for example, of about 1.05. The wire is left in the solution for about 10 seconds, and is placed immediately in water, agitating for a few seconds.

If this does not remove all the oxide, the process may be repeated.

The solutions should be at nearly their boiling point for best results.

When the oxide is all removed, the wire should be rinsed in water.

2

The process is extremely effective, and its action appears to be as follows: After dipping in the nitric acid bath, the metal carries a film of acid over into the hydrochloric acid and momentarily gives a combined solution of great oxidizing power to the formation of free chlorine and chlorine compounds. This lasts only momentarily and the products are soon dispersed in the hydrochloric acid, thereby effectively stopping any further action on the metal itself. My method is therefor self regulating, in that its action stops automatically before corroding the underlying metal appreciably.

The quantity of the second solution in which the metal is dipped, should of course, be very great in comparison with the amount of solution remaining on the metal from being dipped in the first solution.

Although I have described the invention with respect to the foregoing particular embodiment, it is also applicable to other cases where chemical action on a surface is desired and automatic termination of the action is desired before any great penetration of the surface. It may be used where a bath containing a number of ingredients is more effective than a bath of fewer ingredients, so that certain of the ingredients may be present in the first bath, and the remainder in the second.

30 What I claim is:

1. The method of cleaning oxide from an oxidized molybdenum wire, said method comprising: dipping said wire into a solution of nitric acid, removing the wire from said solution, dipping it into a solution of hydrochloric acid while the wire is still wet with the nitric acid solution, removing the wire from said solution and washing the wire with water.

2. The method of claim 1, in which the solutions used are each approximately half acid and half water.

MARIE A. LEVESQUE.

## 45 REFERENCES CITED

The following references are of record in the file of this patent:

## UNITED STATES PATENTS

| 50 | Number    | Name    | Date          |
|----|-----------|---------|---------------|
|    | 145,971   | Sawyer  | Dec. 30, 1873 |
|    | 2,365,153 | Stevens | Dec. 19, 1944 |
|    | 2,410,322 | Weesner | Oct. 29, 1946 |
|    | 2,538,702 | Noble   | Jan. 16, 1951 |